

July 19, 1938.

C. E. GRAY

2,124,294

PRINTING

Original Filed Feb. 12, 1934

Fig. 1



Fig. 2



DESIGN OFFSET FROM  
PENCIL SKETCH OR  
THE LIKE

Fig. 3



Inventor:  
Clyde E. Gray,  
By John J. McLaughlin, C. T. T.

## UNITED STATES PATENT OFFICE

2,124,294

## PRINTING

Clyde E. Gray, Chicago, Ill., assignor of twenty-seven and one-half percent to Marlin Hurt, Chicago, Ill., and twenty percent to McLaughlin & Wallenstein, Chicago, Ill., a partnership composed of John J. McLaughlin and Sidney Wallenstein

Application February 12, 1934, Serial No. 710,895

Renewed December 1, 1937

9 Claims. (Cl. 101—401.1)

My invention relates in general to printing. It relates more in particular to an improved method for reproducing sketches and the like, together with the materials employed in the practice of the method.

It is well-known that there are a large number of methods employed in reproducing one or more negatives of pictures, sketches, and the like, whereby to reproduce such pictures in printed matter. Substantially all methods in common use have their own particular advantages, are most suitable for certain purposes, and in general produce somewhat different effects on the eye. Processes for producing pictures, sketches, and the like, may in general be divided into the class of processes in which plates are produced capable of successfully making a large number of impressions, say on the order of two hundred and fifty thousand, or more; and methods resulting in the production of printing plates which are in general capable of producing a smaller number of impressions, say on the order of twenty five thousand, or thereabouts. For example, etchings and the like typify the former class. The latter class is typified by processes wherein designs are reproduced by wood blocks, by rubber mats and the like. In the latter types of processes, the design is usually cut out by hand, thereby securing certain advantages, but also encountering many disadvantages, as those skilled in the art understand.

The principal object of my present invention is the provision of an improved process for reproducing designs such as pictures, sketches, and the like.

Another object is the provision of a process particularly suited for use when a relatively small number of impressions are desired, but capable of ready adaptation for the purpose of producing a relatively large number of impressions.

Another object is the provision of a printing process of the character described, wherein the reproduction of the printing plate is greatly simplified.

Another object is the provision of an improved material from which to manufacture printing plates of the character used for reproducing designs, sketches, and the like.

Other objects and features of the invention will be apparent as the detailed description progresses.

In the accompanying drawing, I illustrate an embodiment of my invention indicating some of the main steps in the carrying out of my

process in the use of my improved product. In such drawing

Fig. 1 is a perspective view partly broken away showing the printing plate blank used in accordance with my invention, the coating forming a part of the blank being shown relatively thicker for illustration purposes;

Fig. 2 is a plan view of a plate such as shown in Fig. 1, showing the design applied thereon; and

Fig. 3 is a plan view showing the appearance of the plate when completed.

For the convenience of those skilled in the art, I shall first describe a specific and preferred embodiment of my invention, and thereafter shall show the manner in which the same can be modified within the scope of the claims. At this time, I wish to state also that the term "plate" is employed throughout in a general sense to include any type of surface from which designs other than ordinary type are printed, and no limitation as to the character or type of material is to be inferred unless a limitation appears in the context.

The first step in the practice of my invention is the provision of a suitable material from which the printing plates of my invention are to be produced. An extremely satisfactory product is produced by selecting a relatively dense linoleum of conventional type and treating the same to form a very hard but tough and non-friable surface thereon. Several different types of coatings can be employed for the purpose, but in general an oil base enamel prepared to dry with a very hard surface is most suitable for the purpose. While many different types of enamels may be used with success, I have found that unusually good results are obtained if I employ the type of enamel sold by the Sherwin Williams Company under the name of "Enameloid." For reasons which will appear obvious, the coating is preferably white, but I do not limit myself to a strictly white coating. Conventional types of linoleum consisting of a backing of textile material such as canvas and a relatively thick layer consisting essentially of powdered cork and linseed oil can be used. I prefer to use a linoleum having a thickness of approximately an eighth of an inch, and in which the linoleum material is very dense. The linoleum product sold as Armstrong's "Battleship" Linoleum is very suitable.

In producing my plate material, I first dress down the surface of the linoleum to remove all superficial matter such as grease, wax, and the like, and also to produce a very smooth but some-

what porous surface. This step is carried out very satisfactorily by scrubbing with ordinary pumice stone until a perfectly uniform, dull, clean surface is obtained. The linoleum is now allowed to dry until all traces of moisture have been evaporated. The time required for this will vary, depending upon atmospheric conditions. The polished linoleum surface is now covered by applying the "Enameloid" or other suitable coating material to the same, preferably by spraying. The coating should be sufficiently thick to cover the surface thoroughly and leave a perfectly smooth, dense coat; although in general I prefer that the coating not be thick enough to interfere with the flexibility of the linoleum. I find that the best coat is one which is as thin as possible and will still cover the linoleum uniformly and leave a hard finish. After the coating has been applied, it is allowed to set. Here again the time required depends upon conditions. When an enamel is used, I prefer to allow at least one week for the coating to set, but preferably twelve to fourteen days before using the product.

The next step in the operation is transferring the design, such as a sketch, to the hard linoleum coating. This is done by wiping the coating with a material which will cause a very slight softening of the extreme outer surface. I find that a very suitable liquid for this purpose is ordinary alcohol. After the surface has been treated with the alcohol, it is wiped dry and the design in the form of a pencil, ink, or crayon sketch, or in fact made in any of the ways in which original designs are usually produced, is placed flat against the surface and pressure applied thereto to cause the sketch to be applied in reverse onto the surface. To assist in transferring the sketch to the surface of the plate material, the sketch may be burnished with a smooth, blunt instrument and this will cause all of the lines to be transferred to the white surface of the plate material. Another method is to apply the drawing to the surface of the plate material and run the two together between rollers made of a hard substance so as to give a smooth, even pressure that gives approximately the equivalent of burnishing. This method is very satisfactory because it absolutely does away with any slipping between the design and surface against which it is applied and also because the capacity is increased, as, in general, it takes considerably less time to effect the transfer by the latter method.

After the design has been applied to the plate material, portions of the linoleum are cut away to remove that portion which is not intended to be printed. This is done in several different ways, depending upon the design, skill of the operator, and other conditions. In general, the most satisfactory method is to trim the larger portions of the design by means of a machine tool, such as a routing tool, and then to finish up the design by hand. This produces a plate with a raised surface, very suitable for printing and having other advantages as will be pointed out.

If a design is to be reproduced in a number of colors, this is readily taken care of by the method of my invention. I find that the design may be transferred at least three times, and usually as much as seven or eight times, while still giving distinct outlines which are easily followed in cutting the plate. As an example, supposing a design is to be made in green and yellow. In this case, the original artist's drawing will usually be done in green and yellow. Two transfers are made from the same drawing, and in one case the yel-

low portion of the drawing is left in relief and in the second case the green portion is left in relief. In printing, these two plates are registered the same as in any other type of color printing so as to produce the final two-color print.

After the plates have been produced, they are mounted on type-high blocks with wood or metal backs of the type sometimes referred to as a pattern base, in each case as required for use in the particular type of printing equipment employed. For example, the plates can be used on an ordinary flat bed press or they can be used on a rotary press, because the linoleum is of such a character that it will readily take the curve of the roller.

The surfaced linoleum plate of my invention offers considerable advantage in printing over the rubber plates that have been used in some cases in the past and which most closely resemble the plates of my invention. My plates are superior to the rubber plates, first because they require no special attention, they can be used on any type of press, and produce a very clear, clean outline independent of the pressure applied thereto in making the impression.

Printing plates made in accordance with the process outlined above stand up for a considerable length of time, in general, considerably longer than rubber mats, wood blocks, and similar printing surfaces, which the present invention is in large part intended to supplant. However, where a large number of impressions is desired, I can employ the plates of my invention to produce stereotypes or electrotypes directly. To do this, the surfaced linoleum plate is first chilled either in cold water or air to reduce its plasticity. While this chilling is not absolutely necessary, I find that it improves the results sometimes to some considerable extent. A paper mat blank is then laid over the surfaced linoleum plate and a compressible medium laid upon the mat, and the entire assembly placed in a press, according to the usual methods of making a so-called paper mat or other mat usually used in the art. In making a so-called wet mat, it is preferable to place a sheet of foil against the surfaced linoleum plate, then the wet paper on top of the metal foil, after which the usual pressure against a compressible medium is applied to force the paper down into the cut-away portions of the plate. The paper mat may be dried while still in contact with the plate, in accordance with the prevailing custom. The mat so made can be used for producing either stereotypes or electrotypes, or in fact any of the usual plates employed for producing designs.

There are several outstanding advantages in the use of the process of my invention, and other minor advantages which those skilled in the art will understand. In the first place, it furnishes the only process, with which I am familiar, by means of which a printer can make a preliminary run of, say, a few hundred to several thousand, and then, if he wishes to extend the run, he can produce a stereotype from the original plate from which the initial run was made. The process is so simple that within a very short time after a sketch has been produced by an artist, a proof can be run thereof using the same printing plate that would be employed in the printing of a very large number of reproductions.

Another feature of the invention is that it gives a somewhat distinctive effect not found with other printing means and so is capable of producing artistic results not readily possible with other printing processes. This is particularly

true where a large, flat surface is involved. The plate can be made, however, to print very fine lines and for a comparatively short run, good results can be produced. Another advantage 5 is that the method offers a quicker and simpler means of transferring a design and producing a plate therefrom. It also enables the processor to avoid finishing a drawing, as the transfer can be made directly from an original sketch. It 10 offers advantages over such materials as rubber, wood blocks, and the like, because the material is easily routed by machine and it is unnecessary to do all the finishing work by hand. Another advantage is that the materials employed are 15 relatively inexpensive but at the same time do not require any special treatment in the pressroom. For example, the surface can be washed or treated with any substance which is used for washing type and ordinary printing plates, thus 20 affording an advantage over rubber, which must be kept out of contact with many materials found around the ordinary pressroom. The method offers the advantage of many different techniques and effects insofar as the finish thereof is concerned, while at the same time plates, including 25 electrotypes and stereotypes, can be made at considerable saving in cost over methods now commonly used.

I can make several substitutions of materials 30 in carrying out my process and, although results are produced which I do not consider quite as satisfactory as in the preferred method described above, still the method can be used with substituted materials with considerable advantage 35 over methods now in use. In the first place, the surface material employed over the linoleum can be modified extensively. Enamel bonds readily with the linoleum and is preferred for this and other reasons. However, I may employ 40 a very thin sheet of celluloid or other usual cellulose derivative materials capable of being produced in sheet form, and secure the same adhesively to the upper surface of the linoleum. Various types of condensation products may 45 be furnished in sheet form and secured in the same way. I may also employ other types of surfacing materials, such as varnishes made from condensation products, such as phenolic resins, lacquers, special types of hard drying paints, and the like. Considerable difficulty is found, 50 however, in employing the condensation products in obtaining the proper hardness and toughness of the coating. Lacquers and the like can be employed with suitable plasticizing agents and, if 55 used within a comparatively short time, say two or three weeks, good results can be obtained. I find, however, that lacquers tend to become more brittle with age and finally will become unsuited to the purpose.

60 In place of a linoleum made entirely from powdered cork and linseed oil, I may use so-called linoleums containing various types of bonding and filler materials. For example, wood pulp, some earthy materials in pulverulent form, 65 and other substances of this kind are sometimes used as fillers, while in place of linseed oil, and sometimes in addition to the linseed oil, other drying and semi-drying oils can be used. For good results, whatever the composition of the 70 linoleum, it is desirable that it be of substantially the same density and other characteristics of the so-called battleship linoleum, and that it be semi-flexible and capable of comparatively easy cutting with a knife or other tool. Some forms of 75 material containing a great deal of asphalt for

example can be used with fair results. When I use the term "linoleum" therefore I employ it in a broad sense to include true linoleums and linoleum-like products. In addition to linoleum, I can employ other types of base materials, such 5 as sheets made of so-called plastic wood, wood itself, and other types of materials capable of being worked, possessing some toughness, not too brittle, and capable of withstanding sufficient pressure without deforming to permit the manufacture of stereotype mats. In each case, of course, the base material is provided with a tough surface coating to assure the formation of sharp lines for printing, and facilitating the formation 10 of the mats.

15 It is believed that the preceding description is sufficiently clear to enable those skilled in the art to practice the invention. For further clearness, however, the invention will be referred to briefly by reference to the accompanying drawing.

The block shown in Fig. 1 comprises linoleum 10 with an oil base coating 11, preferably white, and a support 12, such as a block of wood, designed to make the surface of the coating type-high. The oil base coating is shown relatively 25 thick but, as previously noted, it should be thick enough to completely cover the linoleum but thin enough so as not to substantially reduce the flexibility thereof. The coating is formed of a 30 paint-like material such as the oil base gloss paint known in the paint trade as "enamel". Non-cellulosic paint-like materials having an oil base readily adherent to the linoleum, which in itself does not resist the wetting action of oil, 35 adhere firmly to the linoleum. This coating has the double function of providing a ready means for the transfer of simple pencil sketches, for example, and of providing a surface which will stand up longer in printing than the usual 40 linoleum surface.

Figs. 2 and 3 illustrate the process of applying the design, and the appearance of the finished plate after the coating and linoleum have been 45 routed out around the design.

I have described my invention in detail so that those skilled in the art may understand how to practice the same and I have also described modifications of my invention which, although not so satisfactory, can be used to reproduce my 50 results on some types of work. My invention, however, is not limited to the matter specifically described, but the scope thereof is set out in the appended claims.

55 As is well known, the term "linoleum" includes compositions comprising a filler, such as cork, a binder, such as oxidized linseed oil, with or without pigments and with or without the conventional backing of canvas or the like. It will be understood that the term "linoleum", as used 60 throughout the specification and claims, possesses this well understood significance.

65 What I claim as new and desire to protect by Letters Patent of the United States is:

1. A method of forming a printing plate which 65 comprises applying a relatively thin oil base coating to a smooth plane surface of linoleum, drying the coating, treating said coating to partially plasticize the surface thereof, pressing a paper on which a design has been drawn against the coating, 70 causing said design to be transferred to the coating, and routing out the design by removing the coating and portion of the linoleum.

2. The method of making a printing plate 75 which comprises applying an oil base coating to

- linoleum, drying the coating, and forming a design in relief by partially cutting away the coating and the linoleum under the same.
3. A printing plate comprising a linoleum base, and a printing surface consisting of a relatively thin oil base coating attached to the base.
4. The method of forming a printing plate which comprises applying to a linoleum surface a light colored oil base coating to provide a hard, dense surface on said linoleum, pressing against the coating a previously prepared design on a cellulosic surface, the design being offset onto said paint-like coating, and routing out the design by removing a portion of the coating and linoleum underneath the same.
5. The method of forming a printing plate which comprises applying a relatively thin coating of white oil base enamel to a linoleum surface, applying a design on the coating by offsetting the same from a paper surface on which the design has been drawn, and routing out the design by removing portions of the coating and underlying linoleum.
6. A printing plate comprising a plane sheet of linoleum provided with a relatively thin adherent

oil base coating, a part of said coating and the linoleum sheet therebeneath being cut away to form a design in relief.

7. A printing plate comprising a linoleum base material provided with an adherent white relatively hard oil base coating, a part of said coating and the base material therebeneath being cut away to form a design in relief. 5

8. A method of forming a printing plate which comprises providing a sheet of linoleum having a relatively hard oil base coating on one surface thereof, treating said coated surface to partially plasticize it, transferring a design upon said plasticized surface, and routing out the design by removing the coating and a portion of the 10 underlying linoleum.

9. A method of forming a printing plate which comprises providing a sheet of linoleum having a white relatively hard oil base coating on one surface thereof, treating said coated surface to 20 partially plasticize it, transferring a design upon said plasticized surface, and routing out the design by removing the coating and a portion of the underlying linoleum.

CLYDE E. GRAY. 25